

May 4, 1943.

E. CZAPEK

2,318,552

PROCESS FOR THE MANUFACTURE OF FILMS, FOILS, BANDS,  
AND THE LIKE FROM CELLULOSE SOLUTIONS

Filed Dec. 17, 1936

Fig.1



Fig.2



Inventor:

Emil Czapek,  
By Czapek & Son,  
Att.,

## UNITED STATES PATENT OFFICE

2,318,552

## PROCESS FOR THE MANUFACTURE OF FILMS, FOILS, BANDS, AND THE LIKE FROM CELLULOSE SOLUTIONS

Emil Czapек, New York, N. Y.

Application December 17, 1936, Serial No. 116,290  
In Germany December 17, 1935

4 Claims. (Cl. 18—57)

This invention relates to a process for the manufacture of films, membranes, bands, sheets and the like from solutions of cuprammonium cellulose.

The principle underlying the manufacture of film-like bands from cellulose solutions by known processes, such as are described in German Patent Nos. 237,152, 249,256, 421,383 and elsewhere, is that the coagulation of the solution, the shaping of the film and the consolidation thereof, are carried out in the same working stage. When working in accordance with the first two of the aforesaid processes, the conversion of the cellulose solution into the film is carried out while freely suspended in the coagulation bath or only lightly supported by guide rollers, which merely serve to protect delicate membranes from breaking. When the last of the aforesaid processes is employed, the film is left on the moulding drum from the time of its formation until the complete penetration of the precipitation liquid.

The progress of the reactions occurring in these processes can scarcely be controlled externally in any way except by alterations in the chemical reagents or alteration of their concentration.

The present invention on the other hand, opens up the possibility of influencing the film during its formation. This is effected in accordance with the invention by dealing separately with the processes occurring during its formation, by means of a method which differs fundamentally from the previously known processes.

Among the objects of the present invention it is aimed to provide an improved process which will permit dividing one of the main reactions thereof into a succession of steps instead of combining them in one sole step, with a view to increasing the output of machines for carrying out this process and thereby to speed up or expedite the operation of such machines for carrying out such processes.

It is still another object of the present invention to provide an improved process whereby certain of the reactions may be divided into successive steps to increase the flexibility of the process to facilitate regulating the same according to the thickness of film to be produced with a certain predetermined uniformity and consistency and according to the ingredients used.

These and other features, capabilities and advantages of the machines for carrying out the process constituting the invention will appear from the subjoined detail description of the

process and of the embodiments of the machine for carrying out the process illustrated in the accompanying drawing, in which

Figure 1 is a diagrammatic elevation of the apparatus made according to one embodiment for carrying out the process; and

Fig. 2 is a similar diagrammatic elevation of an apparatus made according to another embodiment.

10 According to the invention, the cuprammonium cellulose solution is applied in known manner, for example by means of a pouring slot or the like, on a suitable support (drum or endless band). Whereas in accordance with the known processes the solution is then brought to complete solidification and consolidation on this support, and even completely dried out in some cases, in accordance with the present invention only a superficial preliminary coagulation is carried out on the pouring support, just to such a point that the film can be readily detached from the support.

This film, which is still soft and plastic internally and can be made to redissolve, for example by moistening with water, is then passed on further supports, such as conveyor belts or rollers, through a supplementary coagulation bath, in which it can then be subjected to a second precipitating action varying from the preliminary coagulation.

25 The treatment with dilute acids for the purpose of the further consolidation of the film and removal of the copper therefrom, which otherwise takes place in known processes immediately after the coagulation, follows only after this treatment.

30 The purpose of this separate and regulable treatment is manifold. In the manufacture of cellulose films and the like from cuprammonium cellulose solutions the removal of the ammonia at the correct time and to an extensive degree from the coagulated structure plays an important role. If for example the ammonia be entirely removed immediately after pouring out on to the support, i. e., before the coagulation, the film is extremely difficult to detach from the support. The same thing occurs if the coagulation be effected with bath concentrations of dilute liquor, when the required removal of ammonia from the film occurs too rapidly. In both cases the coagulated product becomes brittle in addition, so that when lifted off from the support it breaks and splinters like glass.

35 If on the other hand the ammonia be removed

to an inadequate extent from the solution, the film becomes turbid when subsequently precipitated and treated with acid, so that an opaque product is obtained, which is highly undesirable in the manufacturer of transparent film structures and the like.

These drawbacks are avoided in accordance with the present invention by effecting a preliminary coagulation first of all on the support, which coagulation proceeds to such a degree that the film can be detached from the support. The subsequent second coagulation proper is then adjusted to the ammonia concentration still present in the film in such a way that the ammonia can escape or is removed from the coagulated structure to the desired degree. For this purpose, for the second coagulation a liquor is preferably selected of lower concentration than for the preliminary coagulation, in order to facilitate the diffusion of the ammonia out of the film. With this treatment it is now also possible to interpose short or long intermediate stretches of the web where the ammonia can escape into the air. The use of the word "coagulation" is here to be definitely distinguished from the word "regeneration" which latter is used to characterize only the treatment in which the previously coagulated film is being transformed into a cellulose hydrate.

The process of the present invention first of all enables cuprammonium solutions to be employed having a higher ammonia content than usual, also permits a better and more thorough removal of the ammonia from the coagulated solutions, and finally enables the output of the machines to be considerably increased and the speed of working to be raised, because only a preliminary coagulation now takes place on the same support, on which otherwise the complete coagulation must be carried out in known manner. This takes much less time. The fact that the film is detached from the support in a perfect manner and better than in the known processes is a further advantage which likewise benefits the speed of production.

The invention will now be described with reference to the following example:

A solution of cuprammonium cellulose, containing approximately 6% of cellulose and 7% of ammonia, is spread out by means of a slot nozzle or other suitable spreading device *a* on the cylindrical shell surface of a moulding drum (Fig. 1) or of a moulding belt *b* (Fig. 2). Through the rotation of the horizontally mounted drum *b*, the solution arrives shortly after the spreading in a coagulation bath *c* consisting of a soda lye of 6% strength, through which it is passed within a few seconds. After leaving this bath the film, now superficially coagulated, is detached from the pouring support and passed on to a take-up drum *d* or the like, from where it is passed along on suitable rollers *e* or suitable supports. During this movement the film is first led freely through the air to enable it to give off a part of the ammonia present in the interior and is then dipped into a bath *f* of a soda lye of 3% strength, in which it remains until the precipitation is completed. It then passes into a bath *g* of sulphuric acid of 2% strength for the purpose of regeneration and removal of the copper. The premature removal of the film from the support also permits the stretching of the film after such removal—similarly to the stretch spinning process for rayon—for the purpose of increasing its strength, by giving the take-up drum *d* an advance. Fig. 1 shows the method of working when

a moulding drum is used, and Fig. 2 shows the use of a moulding belt and a special device for obtaining an open air run after the detachment *d*<sub>1</sub> and *d*<sub>2</sub>.

Subsequent to the regenerating and de-copperizing step which may take place in the bath *g* aforesaid, as is customary, the resulting layer will be subjected to further treatment including washing, softening and drying.

10 I claim:

1. A process for the manufacture of films, foils, membranes, bands and the like from solutions of cuprammonium cellulose, which comprises pouring a cellulose solution onto a support, advancing the solution so supported through a preliminary coagulating bath containing an aqueous alkaline solution, subjecting the solution so advanced to a preliminary coagulation while being advanced through such preliminary bath to produce a self-sustaining layer readily detachable

15 from the support, detaching the layer so produced from the support, effecting a final coagulation of the layer so produced in a second bath containing a coagulating fluid of a similar nature to that in the first bath but of a lower concentration than that in the first bath, and thereupon subjecting the layer so produced to further successive treatments including regenerating and de-copperizing, washing and drying.

2. A process for the manufacture of films, foils, membranes, bands and the like from solutions of cuprammonium cellulose, which comprises pouring a cellulose solution onto a support, advancing the solution so supported through a preliminary coagulating bath containing an aqueous alkaline solution and subjecting the solution so advanced to a preliminary coagulation while being advanced through such bath to produce a self-sustaining layer readily detachable from

25 the support, detaching the layer so produced from the support, removing the bulk of the ammonia from the layer so produced and thereby effecting final coagulation of the layer so produced in a second bath containing a coagulating fluid of a similar nature to that in the first bath but of a lower concentration than that in the first bath, and thereupon subjecting the layer so produced to further successive treatments including regenerating and de-copperizing, washing and drying.

3. A process for the manufacture of films, foils, membranes, bands and the like from solutions of cuprammonium cellulose, which comprises pouring a cellulose solution having a relatively high ammonia content approximating its cellulose content onto a support, advancing the cellulose solution so supported through a preliminary coagulating bath containing a dilute soda lye and subjecting the cellulose solution to a preliminary coagulation while advancing through said bath to produce a self-sustaining layer readily detachable from the support, detaching the layer so produced from the support, effecting final coagulation of the layer so produced in a second bath containing a coagulating fluid of similar

35 nature to that in the first bath but of a lower concentration than that in the first bath, and thereupon subjecting the layer so coagulated to further successive treatments including regenerating and de-copperizing, washing and drying.

4. A process for the manufacture of films, foils, membranes, bands and the like from solutions of cuprammonium cellulose, which comprises pouring a cellulose solution onto a support and spreading it thereon while said support and said solution are substantially free of coagulating

40

45

50

55

60

65

70

75

liquids, whereby said spread solution adheres to said support, advancing the cellulose solution so supported through a preliminary coagulating bath, and subjecting the cellulose solution so advanced to a preliminary coagulation while advancing through such bath to produce a partly coagulated layer readily detachable from the support, detaching the layer so produced from the support, passing the layer while being so detached immediately onto a second support having a movable surface disposed closely adjacent to the first

support, moving said surface at a faster rate than said first support to stretch the intervening area of the thus partly coagulated layer disposed between the two supports, thereupon effecting final coagulation of the layer so stretched in a second bath, containing a coagulating fluid of a similar nature to that in the first bath and thereupon subjecting the layer so coagulated to further successive treatments including regenerating and decopperizing, washing and drying.

EMIL CZAPEK.